

**UNITED STATES PATENT OFFICE**

1,968,879

# PROCESS FOR DYEING AND PRINTING TEXTILE MATERIAL

Miles Augustinus Dahlen, Wilmington, and  
Frithjof Zwigmeyer, Gordon Heights, Del., as-  
signors to E. I. du Pont de Nemours & Company,  
Wilmington, Del., a corporation of Delaware

**No Drawing. Application December 3, 1932,  
Serial No. 645,585**

16 Claims. (Cl. 8-5)

This invention relates to processes for dyeing and printing textile material, and more particularly refers to processes for dyeing and printing with compositions comprising an ice color coupling component and a diazoimino compound which is produced by coupling a secondary sugar amine with a diazotized aromatic amine containing no water solubilizing group.

It is an object of this invention to produce dyeings and printings of excellent fastness on textile material. A further object is to produce results which are superior to those obtained with the tedious dyeing and printing processes previously used, by a much simpler method. Additional objects will appear hereinafter.

15 These objects are attained by the present in-  
vention wherein the material to be dyed or print-  
ed is treated with a mixture comprising an ice  
color coupling component and a diazoimino com-  
20 pound which is produced by coupling a secondary  
sugar amine with a diazotized aromatic amine  
containing no water solubilizing group. This di-  
azoimino compound has the following general  
formula:



30 in which "Aryl" represents an aromatic radical which may have substituted thereon non-water-solubilizing groups, R represents an alkyl, aralkyl, or completely reduced carbocyclic radical, and x represents one of the integers 2, 3, 4. The  
 35 color is then developed on the treated material by subjecting it to the action of a weak acid at elevated temperatures.

40 The invention will be more completely understood by reference to the following illustrative examples in which the quantities are stated in parts by weight.

### **Example 1**

7.5 parts of the dry diazoimino compound prepared by the action of methyl-glucamine on di-



55  
was mixed mechanically with 5.03 parts of the  
ortho-toluidide of 2:3-hydroxy-naphthoic-acid.  
To this mixture was added with stirring 3.00  
parts of Turkey red oil, followed by 5.70 parts  
of a 30 per cent solution of sodium hydroxide. 60  
18.77 parts of water heated to 160° F. was next  
added; and when a clear solution was obtained,  
60.00 parts of a neutral starch-gum tragacanth  
thickener was added. The whole was agitated to  
a smooth printing paste. 65  
er

Cotton piece goods were printed from an engraved copper roll with the above paste. The printed fabric was dried in the air, then steamed. 65

A developing bath of the following composition was prepared and heated to 205° F.: 70

|                     | Parts |
|---------------------|-------|
| Glacial acetic acid | 1.0   |
| Formic acid         | 0.5   |
| Glauber's salt      | 2.5   |
| Water               | 96.0  |
|                     | 75    |

The printed and aged fabric was immersed in the bath for about 20 seconds, holding the temperature at 205° F., resulting in the development according to the printed pattern of the dyestuff of the following probable formula:



When color development was complete, the printed fabric was rinsed, soaped with a hot soap solution, again rinsed and dried.

The pattern was developed to a beautiful orange shade, showing excellent fastness to washing, light, and so forth.

#### Example II

A printing paste of the following composition was prepared as in Example No. I.

7.0 parts of the diazoimino compound obtained by the action of diazotized meta-chloroaniline on methyl-galactamine, of the probable formula:



20 2.85 parts of the ortho-toluidide of 2:3-hydroxy-naphthoic-acid  
3.00 parts of sodium hydroxide solution of 30 per cent strength  
25 87.15 parts of neutral thickener

100.00

The fabric was printed and steamed according to the method described in the previous example, and the dyestuff developed by the same procedure. 30 The color formed on the fiber was chemically identical with that obtained according to Example No. I, and the printed pattern was again developed as a beautiful orange of excellent fastness properties.

35

#### Example III

A printing paste of the following composition was prepared:

40 5.4 parts of the diazoimino compound obtained by the action of methyl-glucamine on 4-chloro-2-amino-anisole, of the probable structure:



50 4.6 parts of the ortho-anisidine of 2:3-hydroxy-naphthoic-acid  
3.0 parts of Turkey red oil  
55 5.2 parts of caustic soda solution of 30 per cent strength  
21.8 parts of water—heated to 160° F.  
60.0 parts of neutral thickener, prepared from:

60 100.0

|                                |       |
|--------------------------------|-------|
| Wheat starch-----              | Parts |
| Water-----                     | 60    |
| Gum tragacanth—6 per cent----- | 580   |
|                                | 360   |
|                                | 1000  |

65 Cotton piece goods were printed with the above paste, from an engraved copper roll, the printed material dried and then subjected to the action of live steam containing acetic acid vapors. When color development was complete, the printed fabric was washed with water, treated with a hot soap solution, rinsed and dried. The pattern was 75 developed as a bright red dyeing of excellent fast-

ness properties, the color being due to the development on the fiber of the dyestuff of the probable formula:



#### Example IV

The process of Example No. III was repeated, using a paste of the following composition:

2.7 parts of the reaction product of diazotized 4-chloro-2-amino-anisole and butyl-glucamine, of the probable formula:



10.0 parts of ethyl alcohol  
14.8 parts of water  
2.96 parts of the ortho-anisidine of 2:3-hydroxy-naphthoic-acid  
3.00 parts of caustic soda solution of 30 per cent strength  
66.54 parts of neutral thickener

100.00

The pattern was developed to a bright red, due to the formation of the dyestuff of the formula given in the previous example.

115

#### Example V

A printing paste was prepared of the following composition:

2.7 parts of the diazoimino compound obtained by the action of butyl-xylamine on diazotized 4-chloro-2-amino-anisole, of the following probable formula:



10.0 parts of 2B alcohol  
14.8 parts of water  
2.96 parts of the ortho-anisidine of 2:3-hydroxy-naphthoic-acid  
3.00 parts of sodium hydroxide solution of 30 per cent strength  
66.54 parts of neutral thickener

100.00

The printed fabric was developed without steaming in a bath prepared from:

|                       |       |
|-----------------------|-------|
| Acetic acid 100%----- | Parts |
| Formic acid 85%-----  | 1.0   |
| Sodium sulfate-----   | 0.5   |
| Water-----            | 2.5   |
|                       | 96.0  |
|                       | 100.0 |
|                       | 150   |

the bath being previously heated to 205° F. and held at this temperature during the color development. When the dyestuff was completely formed on the fiber, the cloth was washed, soaped, rinsed and dried. The pattern was developed as a bright red of good fastness properties. The dyestuff was identical with that obtained in the previous example.

*Example VI*

10 A printing paste was prepared from:

3.92 parts of the reaction product of diazotized para-chloro-ortho-toluidine and methyl-glucamine, of the probable formula:



25 4.28 parts of the ortho-phenetidide of 2:3 hydroxy-naphthoic-acid  
3.00 parts of Turkey red oil  
7.00 parts of caustic soda of 30 per cent strength

30 14.80 parts of water heated to 160° F.  
67.00 parts of starch-tragacanth thickener

100.00

35 The cotton piece goods were printed as in the previous example and the dyestuff developed on the fiber by treatment in the acetic-acid-formic-acid-sodium-sulfate bath at 200-210° F. The pattern was developed as a bright scarlet dyeing of excellent fastness properties, the color being 40 due to the formation of the dyestuff of the probable formula:



*Example VII*

55 Equal quantities of the diazoimino compound from diazotized 4-chloro-2-toluidine and methyl-glucamine, of the formula given in the previous example, and the sodium salt of the ortho-phenetidide of 2:3-hydroxy-naphthoic-acid were 60 intimately mixed. A printing paste of the following composition was then prepared:

Mixture of diazoimino compound and ortho-phenetidide of 2:3-hydroxy-naphthoic-acid

Parts

|                                      |       |
|--------------------------------------|-------|
| Water                                | 8.6   |
| Turkey red oil                       | 23.2  |
| Caustic soda of 30 per cent strength | 3.0   |
| Neutral thickener                    | 62.0  |
|                                      | 100.0 |

75 Cotton goods were printed and developed as in the previous example, the same excellent scarlet dyeing being obtained.

*Example VIII*

A printing paste was prepared of the following composition:

|                                                                                                                          |        |
|--------------------------------------------------------------------------------------------------------------------------|--------|
| 4.00 parts of the diazoimino compound from 4-chloro-2-toluidine and methyl-glucamine, of the formula given in Example VI | 80     |
| 3.70 parts of the ortho-toluidide of 2:3-hydroxy-naphthoic-acid                                                          | 85     |
| 3.00 parts of Turkey red oil                                                                                             |        |
| 6.80 parts of caustic soda solution of 30 per cent strength                                                              |        |
| 15.50 parts of water heated to 160° F.                                                                                   |        |
| 67.00 parts of starch-tragacanth thickener                                                                               | 90     |
|                                                                                                                          | 100.00 |

Cotton piece goods were printed with the above paste, from an engraved roll. The printed fabric was then subjected to the action of saturated steam containing the vapors of acetic acid, at a temperature of about 212° F. Rapid development of the pattern to a bright red was effected. When the formation of color was complete, the fabric was rinsed, soaped at the boil, rinsed and dried. The fast red printing had resulted from the formation of the "ice-color" of the probable formula:



*Example IX*

The process of Example No. VIII was repeated, using a paste of the following composition:

|                                                                                                                                                 |     |
|-------------------------------------------------------------------------------------------------------------------------------------------------|-----|
| 2.7 parts of the diazoimino compound obtained by the action of diazotized 4-chloro-2-amino-toluene on methyl-xylamine, of the probable formula: | 120 |
|-------------------------------------------------------------------------------------------------------------------------------------------------|-----|



|                                                                 |        |
|-----------------------------------------------------------------|--------|
| 10.0 parts of ethyl alcohol                                     |        |
| 14.8 parts of water                                             |        |
| 2.96 parts of the ortho-toluidide of 2:3-hydroxy-naphthoic-acid | 135    |
| 3.00 parts of sodium hydroxide of 30 per cent strength          |        |
| 66.54 parts of neutral thickener                                | 140    |
|                                                                 | 100.00 |

As in the previous example, the pattern was developed as a beautiful red dyeing of excellent fastness properties. The dyestuff of the formula given in that example is also formed in this case.

*Example X*

Well-boiled and dried cotton yarn was impregnated with the anilide of 2:3-hydroxy-

150

naphthoic-acid wrung as dry as possible, and immediately developed in the following bath:

5 0 parts of the diazoimino compound obtained by the action of diazotized meta-chloro-aniline on ethyl-glucamine, of the probable formula:



1.0 part of glacial acetic acid  
0.5 part of formic acid  
2.5 parts of Glauber's salt  
91.0 parts of water  
20 100.0

25 The bath was warmed to about 150° F. before immersing the yarn, and the temperature was raised rapidly to about 210° F. The yarn was dyed a bright orange shade, due to the formation of a dyestuff having the following probable formula:



40 After color development was complete, the yarn was rinsed, soaped at the boil, rinsed and dried. The fastness of the dyeing thus obtained is excellent.

45 *Example XI*

50 Cotton piece goods were impregnated with the ortho-toluidide of 2:3-hydroxy-naphthoic-acid in the usual manner. It was dried, then printed from an engraved roll with a paste of the following composition:

55 8 parts of the diazoimino compound obtained by the action of methyl-glucamine on diazotized meta-chloro-aniline, of the formula given in Example No. I  
3 parts of Turkey red oil  
1 part of caustic soda of 30 per cent strength  
23 parts of water  
65 parts of starch-gum tragacanth thickener  
60 100

65 The printed fabric was steamed, then developed by the method described in Example No. I. The printed material was washed in the usual manner to remove uncoupled arylamide, soaped, rinsed and dried. The pattern was produced as an orange dyeing similar to that obtained according to Example No. I, in which the diazoimino compound and the arylamide were both incorporated in the printing paste.

70 Numerous other diazoimino compounds, in addition to those mentioned in the above examples, may also be used in carrying out the process of the present invention. These diazoimino compounds may be prepared from any of the aro-

matic amines commonly used in the ice color art, among which are the following:

75 3-nitro-4-amino-toluene, 2:5-dichloroaniline, 4-chloro-2-amino-toluene, 4-chloro-2-amino-anisol, ortho-chloro-aniline, meta-chloro-aniline, para-nitraniline, 1-amino-4-benzoylamino-2:5-dieoxy-benzene, 4-chloro-2-nitro-aniline, N-(para amino benzoyl)-aniline, ortho-phenetidine-azo-alpha-naphthylamine, para-anisidine-azo-2:5-dimethoxy-aniline, alpha-amino-an-thraquinone, 3-amino-carbazole, dianisidine, para-amino-diphenyl, 4,4'-diamino-diphenylamine, 1-amino-2-methoxy-naphthalene.

80 While any of the aromatic amines shown containing no water-solubilizing groups may be used, better results are usually obtained by selecting amines from the benzene, diphenyl, diphenylamine, naphthalene, azo-benzene, anthraquinone or carbazole series. These amines may have substituted thereon one or more non-water solubilizing groups such as, halogen, alkyl, alkoxy, nitro and benzoyl-amino.

85 To produce the diazoimino compounds the previously mentioned ice color amines are diazotized and coupled with secondary sugar amines, examples of a few of which are:

90 Methyl-glucamine, ethyl-glucamine, cyclohexyl-glucamine, benzyl-xylamine, methyl-erythramine, ethyl galactamine, amyl-arabamine, methyl-mannamine.

95 Preparation of the secondary sugar amines may be carried out by any of the usual processes. For example, the liquid phase catalytic hydrogenation of a mixture of an aldoe of the following general formula:



105 in which x represents one of the integers 2, 3, 4; and a primary amine having the general formula: R-NH<sub>2</sub>

110 in which R represents an alkyl, aralkyl, or completely reduced carbocyclic group. The different optical modifications of the aldoses, namely, the dextro-, laevo-, meso-, and racemic modifications may be used in preparing this secondary sugar amine.

115 The diazoimino compound may then be mixed with one of the usual "ice color" coupling components, such as an arylamide of 2:3-hydroxy-naphthoic acid, an arylamide of hydroxy-carbazole- or hydroxy-naphthocarbazole-carboxylic acid, an arylamide of hydroxy-anthracene-carboxylic acid, alpha- or beta-naphthol, an acetoacetyl derivative of an arylamine, or phenylmethyl pyrazolone. It is to be understood that this mixture may contain one or more diazoimino compounds and one or more "ice color" coupling components, since certain shades are obtained by using more than one diazoimino compound and/or more than one ice color coupling component which could not be obtained otherwise.

120 The textile material is printed or impregnated with this mixture, and then treated with an acid, preferably a weak acid at elevated temperatures, to hydrolyze the diazoimino compound and permit coupling to take place between the regenerated diazo salt and the ice color coupling component. Acetic and/or formic acids have been found to give very satisfactory results but the invention is not limited to these acids since hydrolysis of the diazoimino compound may be effected by numerous other acids or mixtures of acids, well known to one skilled in the art. The acid or acids used in treating the printed or impregnated

textile material may be in either the liquid or vapor phase.

It is to be understood that the ice color coupling component or components and the diazoimino compound or compounds need not be applied to the textile material simultaneously, but one may be applied prior to the other, the resulting reaction being fundamentally the same regardless of the order in which the reactants are applied.

It is also to be understood that when reference is made to a mixture of an ice color coupling component and a diazoimino compound this mixture may contain various assistants such as starch, gum, alkali, and Turkey red oil. The compositions of these printing and dyeing mixtures are so well known that no difficulty should be encountered in selecting the proper assistants for any given purpose, in the event that assistants are required.

The process described in the present disclosure produces excellent dyeings and printings on textile material in a much more simplified manner than was previously possible. The colors produced are exceptionally uniform and fast, due in great part to the thorough impregnation of the fibers with the very soluble diazoimino compound. No deleterious side reactions take place to impair the efficiency of the process and the appearance and properties of the products produced. The secondary sugar amine, produced upon hydrolysis of the diazoimino compound, does not have a strong reducing effect, consequently, it does not reduce the diazo salt or interfere in any manner with the coupling of this diazo salt and the ice color coupling component. The compounds used are readily available at a very reasonable cost, and in addition the simplification of the printing or dyeing processes results in an appreciable saving to the manufacturer.

As many apparently widely different embodiments of this invention may be made without departing from the spirit and scope thereof, it is to be understood that we do not limit ourselves to the foregoing examples or description except as indicated in the following claims.

We claim:

1. A process for coloring material which comprises treating the material with a mixture comprising an ice color coupling component and a diazoimino compound, produced by coupling a secondary sugar amine with a diazotized aromatic amine containing no water-solubilizing group, then developing the color by subjecting the treated material to the action of a weak acid at elevated temperatures.

2. A process for coloring material which comprises treating the material with a mixture comprising an ice color coupling component and a diazoimino compound having the following general formula:



in which Aryl represents the residue of an aromatic amine containing no water-solubilizing group, and Z represents the residue of a secondary sugar amine, then developing the color by subjecting the treated material to the action of a weak acid, preferably at elevated temperatures.

3. A process for coloring material which comprises treating the material with a mixture comprising an ice color coupling component and a

diazoimino compound having the following general formula:



80

85

90

95

100

105

110

115

120

125

130

135

140

145

150

in which Aryl represents the residue of an arylamine which may have non-water-solubilizing groups substituted thereon, R represents an alkyl, aralkyl, or completely reduced carbocyclic radical, and x represents one of the integers 2, 3, 4, then developing the color by subjecting the treated material to the action of a weak acid, preferably at elevated temperatures.

4. A process for coloring material which comprises treating the material with a mixture comprising an ice color coupling component and a diazoimino compound having the following general formula:



in which Aryl represents the residue of an arylamine of the benzene, diphenyl, naphthalene, diphenylamine, azobenzene, anthraquinone or carbazole series, which may have non-water-solubilizing groups substituted thereon, R represents an alkyl, aralkyl, or completely reduced carbocyclic radical, and x represents one of the integers 2, 3, 4, then developing the color by subjecting the treated material to the action of a weak acid, preferably at elevated temperatures.

5. A process for coloring material which comprises treating the material with a mixture comprising an ice color coupling component selected from the group consisting of arylamides of 2-3-hydroxy-naphthoic acid, arylamides of hydroxy-carbazole- or hydroxy-naphthocarbazole-carboxylic acids, arylamides of hydroxy-anthracene-carboxylic acids, alpha- or beta-naphthol, acetoacetyl derivatives of arylamines, and phenylmethyl-pyrazolone, and a diazoimino compound having the following general formula:



in which Aryl represents the residue of an arylamine of the benzene, diphenyl, naphthalene, diphenylamine, azobenzene, anthraquinone, or carbazole series, which may have non-water-solubilizing groups substituted thereon, R represents an alkyl, aralkyl, or completely reduced carbocyclic radical, and x represents one of the integers 2, 3, 4, then developing the color by subjecting the treated material to the action of a weak acid at elevated temperatures.

6. A process for coloring material which comprises treating the material with a mixture comprising an ice color coupling component selected from the group consisting of arylamides of 2-3-hydroxy-naphthoic acid, arylamides of hydroxy-carbazole- or hydroxy-naphthocarbazole-carboxylic acids, arylamides of hydroxy-anthracene-carboxylic acids, alpha- or beta-naphthol, acetoacetyl derivatives of arylamines, and phenylmethyl-pyrazolone, and a diazoimino compound having the following general formula:



in which Aryl represents the residue of an aryl-

amine of the benzene, diphenyl, naphthalene, diphenylamine, azobenzene, anthraquinone, or carbazole series, which contains no water-solubilizing group but which may have substituted

5 thereon members selected from the group consisting of halogen, alkyl, alkoxy, nitro and benzoylamino; R represents an alkyl, aralkyl, or completely reduced carbocyclic radical, and x represents one of the integers 2, 3, 4, then developing

10 the color by subjecting the treated material to the action of a weak acid at elevated temperatures.

7. A process for coloring material which comprises treating the material with a mixture comprising an arylamide of 2-3-hydroxy-naphthoic acid having the following general formula:



in which R represents the residue of an arylamine of the benzene or naphthalene series which may have non-water-solubilizing groups substituted thereon, and a diazoimino compound having the following general formula:



in which Aryl represents the residue of an arylamine of the benzene or naphthalene series which may have substituted thereon non-water-solubilizing groups, R represents an alkyl, aralkyl, or completely reduced carbocyclic radical, and x represents one of the integers 2, 3, 4, then developing the color by subjecting the treated material to the action of an acid selected from the group consisting of acetic and formic acid, at elevated temperatures.

8. A process for coloring material which comprises treating the material with a mixture comprising an arylamide of 2-3-hydroxy-naphthoic acid having the following general formula:



in which X and Y represent hydrogen, halogen, alkyl or alkoxy groups, and a diazoimino compound having the following general formula:



in which Aryl represents the residue of an arylamine of the benzene series, which may have substituted thereon members selected from the class consisting of halogen, alkyl, alkoxy, nitro and benzoyl-amino groups, R represents an alkyl group, and x represents one of the integers 2, 3, 4, then developing the color by subjecting the treated material to the action of an acid selected from the group consisting of acetic and formic acid, at elevated temperatures.

9. A composition of matter which comprises an ice color coupling component and a diazoimino compound having the following general formula:



in which Aryl represents the residue of an aromatic amine containing no water-solubilizing

group, and Z represents the residue of a secondary sugar amine.

10. A composition of matter which comprises an ice color coupling component and a diazoimino compound having the following general formula: 80



in which Aryl represents the residue of an arylamine which may have non-water-solubilizing groups substituted thereon, R represents an alkyl, aralkyl, or completely reduced carbocyclic radical, and x represents one of the integers 2, 3, 4. 85

11. A composition of matter which comprises an ice color coupling component and a diazoimino compound having the following general formula:



in which Aryl represents the residue of an arylamine of the benzene, diphenyl, naphthalene, diphenylamine, azobenzene, anthraquinone or carbazole series, which may have non-water-solubilizing groups substituted thereon, R represents an alkyl, aralkyl, or completely reduced carbocyclic radical, and x represents one of the integers 2, 3, 4. 100

12. A composition of matter which comprises an ice color coupling component selected from the group consisting of arylamides of 2-3-hydroxy-naphthoic acid, arylamides of hydroxy-carbazole- or hydroxy-naphthocarbazole-carboxylic acids, arylamides of hydroxy-anthracene-carboxylic acids, alpha- or beta-naphthol, aceto-acetyl derivatives of arylamines, and phenylmethyl-pyrazolone; and a diazoimino compound having the following general formula:



in which Aryl represents the residue of an arylamine of the benzene, diphenyl, naphthalene, diphenylamine, azobenzene, anthraquinone or carbazole series, which may have non-water-solubilizing groups substituted thereon, R represents an alkyl, aralkyl, or completely reduced carbocyclic radical, and x represents one of the integers 2, 3, 4. 120

13. A composition of matter which comprises an ice color coupling component selected from the group consisting of arylamides of 2-3-hydroxy-naphthoic acid, arylamides of hydroxy-carbazole- or hydroxy-naphthocarbazole-carboxylic acids, arylamides of hydroxy-anthracene-carboxylic acids, alpha- or beta-naphthol, aceto-acetyl derivatives of arylamines, and phenylmethyl-pyrazolone, and a diazoimino compound having the following general formula:



in which Aryl represents the residue of an arylamine of the benzene, diphenyl, naphthalene, diphenylamine, azobenzene, anthraquinone, or carbazole series, which contains no water-solubilizing group but which may have substituted thereon members selected from the group consisting of halogen, alkyl, alkoxy, nitro and benzoyl-amino; R represents an alkyl, aralkyl, or completely reduced carbocyclic radical, and x represents one of the integers 2, 3, 4. 145

duced carbocyclic radical, and  $x$  represents one of the integers 2, 3, 4.

14. A composition of matter which comprises an arylamide of 2-3-hydroxy-naphthoic acid having the following general formula:



10 in which R represents the residue of an aryl-amine of the benzene or naphthalene series which may have non-water-solubilizing groups substituted thereon, and a diazoimino compound hav-

15 ing the following general formula:



20 in which Aryl represents the residue of an aryl-amine of the benzene or naphthalene series which may have substituted thereon non-water-solubilizing groups, R represents an alkyl, aralkyl, or completely reduced carbocyclic radical, and  $x$

25 represents one of the integers 2, 3, 4.

15. A composition of matter which comprises an arylamide of 2-3-hydroxy-naphthoic acid having the following general formula:



30

35

40

45

50

55

60

65

70

75

in which X and Y represent hydrogen, halogen, alkyl or alkoxy groups, and a diazoimino compound having the following general formula:



80

85

90

95

100

105

110

115

120

125

130

135

140

145

150

in which Aryl represents the residue of an aryl-amine of the benzene series, which may have substituted thereon members selected from the class consisting of halogen, alkyl, alkoxy, nitro and benzoylamino groups, R represents an alkyl group, and  $x$  represents one of the integers 2, 3, 4.

16. A composition of matter which comprises a member selected from the group consisting of the o-toluidide-, and the o-aniside of 2-3-hydroxy-naphthoic acid, and a diazoimino compound having the following general formula:



in which X represents hydrogen or an alkyl or 105  
alkoxy group.

MILES AUGUSTINUS DAHLEN.  
FRITHJOF ZWILGMEYER.